

1

3,053,691

### PROTECTIVE COATING

Harry J. Hartman and Walter E. Pocock, Baltimore Md., assignors to Allied Research Products, Incorporated, Baltimore, Md., a corporation of Maryland  
No Drawing. Filed Jan. 29, 1958, Ser. No. 711,777  
14 Claims. (Cl. 117—75)

This invention relates to the treatment of metals to provide the same with a protective corrosion-resistant and abrasion-resistant coating which also has excellent paint bonding characteristics and, more particularly, to an improved coating composition and method for forming the coating.

A simplified flow diagram of the process is as follows:



Previously used organic coatings necessitate the use of organic solvents and where water soluble resins are used, lack the corrosion protective value, wide range of surfaces which can be successfully coated, and adhesion characteristics covered in this invention.

An object of this invention is to provide metals and alloys thereof, such as steel, aluminum, zinc, cadmium, magnesium, silver, copper, etc., and chemical conversion coatings, e.g., chromate, phosphate and oxide coatings, on these metals with a clear abrasion-resistant and corrosion-resistant protective film, which can be used as a final finish and which provides an excellent base for subsequent painting. This is accomplished by using a water soluble resin, i.e., polyacrylamide with suitable corrosion

2

inhibitor or inhibitors, to coat such metals. It is within the scope of this invention that the polyacrylamide can be added directly to the solution used for generating a chromate conversion coating on the metal surface, co-depositing with the chromate coating. This aspect of the invention is limited in application to metals upon which a conversion coating can be formed. The corrosion resistance, water repellency, and paint bonding characteristics are thereby improved.

10 A further object of this invention is to provide a corrosion protective film on metals and alloys which, if desired, can be removed quickly and easily by immersion in a hot alkaline solution; retaining the clean oxide-free surface available as it was prior to treatment. This is particularly important where a temporary protective film is desired.

15 The invention further comprehends the use of polyacrylamide plus a corrosion inhibitor or inhibitors in aqueous solution as a simple dip brush or spray operation whereby a coating can be applied to a metal surface or to a surface having a previously formed conversion coating, without any objectionable chemical reaction taking place on the surface.

20 It is possible by use of this invention to use organic and inorganic coloring agents to add color to the film.

25 Still further objects and the entire scope of applicability of the present invention will become apparent from the detailed description given hereinafter; it should be understood, however, that the detailed description and 30 specific examples, while indicating preferred embodiments of the invention, are given by way of illustration only, since various changes and modifications within the spirit and scope of the invention will become apparent to those skilled in the art from this detailed description.

35 While a polyacrylamide coating on the metal by itself has little water resistance and a chromate coating by itself, likewise, has little water resistance, it has been found that if a mixture of the polyacrylamide and chromate is employed under acid conditions, the coating obtained has outstanding water resistance. The film is insolubilized simply by drying in open air at room temperature, although the insolubilization procedure can be accelerated by hot drying.

40 We find that polyacrylamide itself possesses little or 45 no corrosion protective value over metals, but, surprisingly, when a corrosion inhibitor or inhibitors are combined with the polyacrylamide, there results a greatly improved corrosion protection over the use of the corrosion inhibitors alone, as well as the polyacrylamide, so that 50 the condition is remedied. In addition, it has been found that by utilizing the polyacrylamide with the corrosion inhibitor, a greatly reduced amount of corrosion inhibitor can be employed to obtain the same amount of protection.

55 In brief, the principal components of the coating which form the subject of the present invention are soluble in acid solutions.

56 The preferred corrosion inhibitor, or inhibitors, used in this invention are water soluble chromium compounds such as chromic acid, sodium, potassium, ammonium dichromate, and the corresponding chromates, as well as less soluble complex chromium-chromate gels containing both hexavalent and trivalent chromium, made, for example, by adding sodium chromate to chromium nitrate under slightly alkaline conditions, and very slightly soluble chromium compounds such as zinc chromate and strontium chromate. Such compounds are excellent cor-

rosion inhibitors when used in conjunction with the polyacrylamide in accomplishing the scope of the invention.

When used as a supplementary coating, the polyacrylamide and inhibitors previously mentioned can be mixed dry and then dissolved in water at the time of application to the metal or they can be premixed with water. The aqueous mixtures can have a pH of 1 to 11, desirably on the acid side, and preferably pH 1 to 3. To maintain the pH, there can be used any acid or acid salt or alkali or alkali salt that does not reduce the chromate too rapidly for practical application. Typical acids which can be employed are hydrochloric acid, sulfuric acid, nitric acid, phosphoric acid, acetic acid, formic acid, chromic acid, etc., and as alkalis there can be utilized sodium, potassium or ammonium hydroxide, or carbonates, such as sodium and potassium carbonates.

The invention also includes the addition of polyacrylamide directly to baths employed for the formation of the chromate conversion coatings. Corrosion resistance, paint bonding characteristics and abrasion resistance are thereby improved. Chromate conversion coatings referred to here are formed by immersion of a metal in a solution comprising hexavalent chromium compounds, and an activator or activators in an acid solution. The metal is dissolved at the interface, the reaction with the metal resulting in a chromate gel which is precipitated on the surface. When polyacrylamide is incorporated in the formulation this is coprecipitated with the chromate gel improving the characteristics, e.g., corrosion resistance, paint bond properties and abrasion resistance, of the film formed.

In what follows, unless otherwise indicated, all parts and percentages are by weight.

The aqueous compositions of the present invention contain 0.05 to 5 parts of polyacrylamide per 100 parts of water. If the polyacrylamide is the film former, as previously described, then it is used in an amount of 0.2 to 5 parts per 100 parts of water. The chromate or other corrosion inhibitor is used in admixture with the polyacrylamide in the amount of 0.01 to 10 parts of inhibitor per 100 parts of water.

If the chromate conversion bath is the primary film former, then only 0.05 to 1 part of polyacrylamide is normally used per 100 parts of water in the aqueous mixture containing 0.01 to 50 parts of chromate as hexavalent chromium.

One of the advantages of the instant invention is that the compositions are relatively low in cost.

Temperatures of 60 to 100° F. are preferably employed in the coating process. Temperatures as high as 200° F. can be employed, however. It is surprising that such high temperatures can be used since it would be expected that there would be quantitative decomposition of the polyacrylamide in the presence of acidified chromates, a strong oxidizing system, at elevated temperatures, e.g., 180° F.

Accelerated drying can be carried out at 120 to 250° F., preferably 140 to 180° F. When acid solutions of polyacrylamide are employed, the drying insolubilizes the film, particularly if the solution is applied over a chromate conversion coating.

The polyacrylamide used in this invention is usually of such a molecular weight range that a 4% aqueous solution has a viscosity varying from 60 to 600 centipoises at 77° F., and preferably 100 to 250 centipoises under these conditions. In the following examples, the polyacrylamide used has a viscosity of 200 centipoises at 77° F. at a 4% concentration.

As dry compositions, there can be used mixtures of polyacrylamide and inhibitor or inhibitors in the following proportions:

|                | Parts      |
|----------------|------------|
| Polyacrylamide | 100        |
| Inhibitors     | 0.2 to 100 |

or mixtures of polyacrylamide and chromate conversion composition mixtures in the following proportions:

|                      | Parts     |
|----------------------|-----------|
| Polyacrylamide       | 0.1 to 50 |
| Chromate composition | 100       |

#### Example 1

A steel test panel electroplated with zinc and at room temperature was immersed in the following aqueous solution having a temperature of 80° F. and immediately withdrawn, the panel being covered with liquid and then dried at 160° F.

|    |                                |         |     |
|----|--------------------------------|---------|-----|
| 15 | Polyacrylamide                 | percent | 2   |
|    | Chromic acid, CrO <sub>3</sub> | do      | 0.2 |
|    | pH                             |         | 2   |

A clear abrasion-resistant coating was formed. The test panel showed only slight edge corrosion after 68 hours' exposure in a standard 20% salt spray. A similar panel, zinc plated only, was severely corroded after 24 hours' salt spray exposure.

#### Example 2

25 Example 1 was repeated using half the specified concentration. Corrosion in salt spray was slightly less than with Example 1, but still an improvement over zinc plate alone.

#### Example 3

30 Example 1 was repeated using double the specified concentrations. Corrosion in salt spray was somewhat greater than with Example 1.

#### Example 4

35 A steel panel was zinc plated, rinsed with water, immersed in the following aqueous solution at 80° F. and then dried at 160° F..

|    |                                                                                      |         |     |
|----|--------------------------------------------------------------------------------------|---------|-----|
| 40 | Polyacrylamide                                                                       | percent | 2   |
|    | Sodium bichromate, Na <sub>2</sub> Cr <sub>2</sub> O <sub>7</sub> .2H <sub>2</sub> O | do      | 0.2 |
|    | pH                                                                                   |         | 6   |

45 A clear abrasion-resistant coating was formed. After 24 hours' salt spray, the panel was only slightly corroded as compared to severe corrosion on a similar panel that was zinc plated only.

#### Example 5

50 A steel panel was zinc plated, rinsed with water and subjected to the following procedure:

(1) Immersed for 20 seconds, at 80° F., in an aqueous solution containing:

|    |                                                                                      |         |      |
|----|--------------------------------------------------------------------------------------|---------|------|
| 55 | Chromic acid, CrO <sub>3</sub>                                                       | percent | 0.1  |
|    | Sodium bichromate, Na <sub>2</sub> Cr <sub>2</sub> O <sub>7</sub> .2H <sub>2</sub> O | do      | 0.3  |
|    | Sulfuric acid                                                                        | do      | 0.28 |
|    | Nitric acid                                                                          | do      | 1.5  |
| 60 | pH                                                                                   |         | 0.2  |

(2) Rinsed with water,  
(3) Immersed in the solution of Example 4, and  
(4) Dried at 160° F.

A clear abrasion-resistant coating was formed. After 120 hours' salt spray exposure, the panel treated by steps 1-4 was markedly less corroded than a panel that had been treated by steps 1, 2, and 4 only. Steps 1, 2, and 4 are an example of a typical commercial chromate conversion treatment designed to improve the corrosion resistance of zinc surfaces.

#### Example 6

An aluminum test panel of 3003 alloy was cleaned, 75 immersed in the solution of Example 4, and dried at

160° F. A clear abrasion-resistant coating was formed. After 66 hours' salt spray exposure, the panel was markedly less corroded than a similar panel that had been cleaned only.

*Example 7*

An aluminum test panel of 3003 alloy was subjected to the following procedure:

|                                                                           |         |       |
|---------------------------------------------------------------------------|---------|-------|
| (1) Cleaned,                                                              | percent | 0.05  |
| (2) Rinsed with water,                                                    | do      | 0.01  |
| (3) Immersed for 3 minutes, at 80° F., in an aqueous solution containing: |         |       |
| Chromic acid, CrO <sub>3</sub>                                            | percent | 0.05  |
| Potassium ferricyanide, K <sub>3</sub> Fe(CN) <sub>6</sub>                | do      | 0.01  |
| Sodium fluosilicate, Na <sub>2</sub> SiF <sub>6</sub>                     | do      | 0.014 |
| Barium nitrate                                                            | do      | 0.02  |
| pH                                                                        |         | 2.5   |

- (4) Rinsed with water,
- (5) Immersed in the solution of Example 4, and
- (6) Dried at 160° F.

A clear abrasion-resistant coating was formed. After 120 hours' salt spray exposure, the panel was markedly less corroded than a similar panel that had been treated by steps 1, 2, 3, 4, and 6 only. Steps 1, 2, 3, 4 and 6 are an example of a typical commercial chromate conversion treatment designed to improve the corrosion resistance of aluminum surfaces.

*Example 8*

A steel panel was cleaned and immersed in the following aqueous solution at 80° F. and dried at 160° F.:

|                                                   | Percent |
|---------------------------------------------------|---------|
| Polyacrylamide                                    | 2       |
| Sodium chromate, Na <sub>2</sub> CrO <sub>4</sub> | 1       |

A clear abrasion-resistant coating was formed. After 1 hour salt spray exposure, the panel was only slightly rusted, as compared to severe rusting of a similar panel that had been cleaned only.

*Example 9*

Example 8 was repeated, using double the specified concentrations. The resistance to rust in salt spray was somewhat greater than with Example 8.

*Example 10*

To one liter of an aqueous acidic solution for passivating and improving the corrosion resistance of zinc surfaces and containing 10 grams of Na<sub>2</sub>Cr<sub>2</sub>O<sub>7</sub>·2H<sub>2</sub>O, 10 grams of H<sub>3</sub>BO<sub>3</sub>, 2.3 grams of NaCl and 1 ml. of 42° Bé. HNO<sub>3</sub> was added 2 grams of polyacrylamide.

A hot-dipped galvanized zinc sheet was immersed in this bath 5 seconds at 140° F. and then dried at 70° F. The coating obtained had improved corrosion resistance as determined by humidity tests, compared to a similar coating from which the polyacrylamide was omitted.

*Example 11*

Example 10 was repeated utilizing 0.25 gram of the polyacrylamide. Corrosion resistance was less than that obtained in Example 10; however, there was a measurable improvement over the coating from which the polyacrylamide was omitted.

*Example 12*

Example 10 was repeated utilizing 5 grams of polyacrylamide with comparable results. Polyacrylamide can be added as above indicated to any of the formulations disclosed in Hartman Patent No. 2,799,601. The performance of said formulations is improved by the polyacrylamide addition.

*Example 13*

An aluminum test panel of 3003 alloy was subjected to the following procedure:

|    |                                                                           |         |      |
|----|---------------------------------------------------------------------------|---------|------|
| 5  | (1) Cleaned,                                                              | percent | 0.2  |
| 10 | (2) Rinsed with water,                                                    | do      | 0.04 |
|    | (3) Immersed for 3 minutes, at 80° F., in an aqueous solution containing: |         |      |
| 15 | Chromic acid, CrO <sub>3</sub>                                            | percent | 0.2  |
|    | Potassium ferricyanide, K <sub>3</sub> Fe(CN) <sub>6</sub>                | do      | 0.04 |
|    | Sodium fluosilicate, Na <sub>2</sub> SiF <sub>6</sub>                     | do      | 0.05 |
|    | Barium nitrate                                                            | do      | 0.08 |
|    | Polyacrylamide                                                            | do      | 0.1  |
|    | pH                                                                        |         | 1.9  |

- (4) Rinsed with water,
- (5) Dried at room temperature.

The panel was then painted with a white baked enamel, along with a panel similarly treated, except that the polyacrylamide was eliminated from the solution of step 20 3. The adherence of the paint to the metal surface was markedly improved by the presence of polyacrylamide as compared to no polyacrylamide.

After 500 hours' salt spray exposure, there was noticeably less corrosion of the metal and less blistering and 25 flaking of the paint where polyacrylamide was included as compared to no polyacrylamide, indicating the beneficial effect of polyacrylamide on corrosion resistance.

*Example 14*

30 Example 13 was repeated except using 0.5% polyacrylamide instead of 0.1%. There was a further improvement in initial paint adherence and in corrosion resistance as indicated by 500 hours' salt spray exposure.

Referring to Examples 13 and 14, polyacrylamide can 35 be profitably added to any of the formulations disclosed in Ostrander et al. Patent No. 2,796,371.

*Example 15*

Zinc metal sheet was dipped into an aqueous solution 40 containing:

|                                |                |
|--------------------------------|----------------|
| Chromic acid, CrO <sub>3</sub> | 7 grams/liter. |
| Sodium sulfate                 | 1 gram/liter.  |
| Nitric acid, 42° Bé.           | 3 ml./liter.   |
| pH                             | 0.3.           |

45 The sheet was allowed to remain in the solution until a visible conversion coating was formed (about 15 seconds). The sheet was then removed, rinsed in water and immersed in an aqueous solution containing:

|                            |                |
|----------------------------|----------------|
| Polyacrylamide             | 2.0%.          |
| Hydrochloric acid, 20° Bé. | 1.7 ml./liter. |

The sheet was then dried at 160° F. A clear water-resistant coating was formed which was superior in abrasion resistance to the conversion coating itself.

*Example 16*

Example 1 was repeated but the aqueous polyacrylamide solution was maintained at 160° F. The results 60 obtained were similar to those in Example 1.

We claim:

1. A composition containing 0.05 to 5 parts of polyacrylamide and 0.01 to 10 parts of a hexavalent chromium compound.
- 65 2. A composition according to claim 1 wherein the chromium compound is present in an amount of 0.05 to 0.5 part.
3. An aqueous composition containing 0.05 to 5 grams 70 of polyacrylamide and 0.01 to 10 grams of a hexavalent chromium compound per 100 parts of water.
4. A composition according to claim 3 having a pH of not more than 5.
- 75 5. A method of imparting a corrosion-resistant coating to a metal which comprises subjecting the metal to an

aqueous solution containing polyacrylamide and a hexavalent chromium compound.

6. A method according to claim 8 wherein the polyacrylamide is present in an amount of 0.5 to 50 grams per liter of solution and the hexavalent chromium compound is present in an amount of 0.1 to 100 grams per liter of solution.

7. A method according to claim 6 wherein the solution has a pH not greater than 5.

8. A method of imparting increased abrasion resistance to a metal having a coating containing a hexavalent chromium compound as a corrosion inhibitor comprising subjecting the metal having said initial coating to an aqueous solution containing polyacrylamide and a hexavalent chromium compound.

9. A method according to claim 8 wherein the polyacrylamide is present in an amount of 0.5 to 50 grams per liter of solution and the hexavalent chromium compound is present in an amount of 0.1 to 100 grams per liter of solution.

10. A method of imparting increased abrasion resistance to a metal having a corrosion-resistant chromate conversion initial coating comprising subjecting the metal having said initial coating to an aqueous solution containing polyacrylamide.

11. A method according to claim 10 wherein the polyacrylamide is present in an amount of 0.5 to 50 grams per liter of solution.

12. A method of imparting a corrosion-resistant coat-

ing to a metal which comprises subjecting the metal to an aqueous solution containing polyacrylamide and a hexavalent chromium compound and thereafter drying the coated metal.

5 13. A method according to claim 12 wherein the aqueous solution has a pH not greater than 5.

14. A method of imparting increased abrasion resistance to a metal having a corrosion-resistant chromate conversion initial coating comprising subjecting the metal having said initial coating to an aqueous solution containing polyacrylamide and thereafter drying.

#### References Cited in the file of this patent

#### UNITED STATES PATENTS

|    |           |            |       |               |
|----|-----------|------------|-------|---------------|
| 15 | 2,335,962 | Pollack    | ----- | Dec. 7, 1943  |
|    | 2,411,590 | Powell     | ----- | Nov. 26, 1946 |
|    | 2,412,528 | Morrell    | ----- | Dec. 10, 1946 |
|    | 2,508,717 | Jones      | ----- | May 23, 1950  |
| 20 | 2,636,257 | Ford       | ----- | Apr. 28, 1953 |
|    | 2,709,664 | Evans      | ----- | May 31, 1955  |
|    | 2,744,080 | Brant      | ----- | May 1, 1956   |
|    | 2,902,390 | Bell       | ----- | Sept. 1, 1959 |
|    | 2,921,858 | Hall       | ----- | Jan. 19, 1960 |
| 25 | 2,930,106 | Wrotnowski | ----- | Mar. 29, 1960 |

#### OTHER REFERENCES

Schildkrecht: Vinyl and Related Polymers, John Wiley and Sons, Inc. (1952), pages 314-317.